

April 29, 1924.

1,491,846

R. G. COATES

STEEL PROCESS, MOLD, AND INGOT

Filed Oct. 6, 1920

2 Sheets-Sheet 1



*Fig. 1.*



*Fig. 2.*



*Fig. 3.*



*Fig. 4.*



Inventor  
Ray G. Coates  
Attorney  
George Ramsey

April 29, 1924.

1,491,846

R. G. COATES

## STEEL PROCESS, MOLD, AND INGOT

Filed Oct. 6, 1920

2 Sheets-Sheet 2



Fig. 6.



Fig. 7.

By

Inventor  
Ray J. Coates  
Attorney  
George Ramsey

## UNITED STATES PATENT OFFICE.

RAY G. COATES, OF PASADENA, CALIFORNIA, ASSIGNOR TO VALLEY MOULD AND IRON CORPORATION, OF SHARPSVILLE, PENNSYLVANIA, A CORPORATION OF NEW YORK.

## STEEL PROCESS, MOLD, AND INGOT.

Application filed October 6, 1920. Serial No. 415,089.

To all whom it may concern:

Be it known that I, RAY G. COATES, a citizen of the United States, and a resident of the city of Pasadena, in the county of 5 Los Angeles, State of California, have invented new and useful Improvements in Steel Processes, Molds, and Ingots, of which the following is a specification.

This invention relates broadly to metallurgy and more particularly to a method and apparatus for casting steel ingots in a covered mold.

More especially the present invention relates to casting steel ingots in a chill mold 15 and comprises a method and apparatus for localizing "blow holes" in the middle of the ingot.

An important object of the present invention is the method of casting steel ingots 20 in a covered mold and causing the "blow hole" bubbles to be trapped in the middle of the ingot a sufficient distance from the surfaces of the ingot to prevent the cavities from breaking out during rolling.

25 A further object of the present invention is a method and apparatus for casting steel ingots having all sides thereof chilled and wherein bubbles are trapped in the middle of the ingot a sufficient distance from 30 the surfaces of the ingot to prevent the cavities from breaking out during rolling.

A still further object of the present invention is a method and apparatus for casting steel ingots having all sides thereof 35 chilled and wherein bubbles are trapped in the middle of the ingot in such manner that the cavities caused by the bubbles will weld together during rolling operations.

Another further and important object of 40 the present invention is a method and apparatus for casting steel ingots in a covered chill mold by providing a substantially horizontal mold arranged with trunnions which rest upon suitable tracks or supports so that the ingot may be released by inverting the mold and freeing the cover.

A still further and important object of 45 the present invention is the method of casting steel ingots which comprises pouring molten steel into a covered chill mold, permitting a solidified cup to form, continuing

the pouring until the metal contacts with the chilled top, thereby sealing said cup, and then inverting the mold and causing gas bubbles to be sealed against the bottom of 55 the originally formed cup.

A still further object of the present invention is a method and apparatus for casting steel ingots wherein zones of isocrystallization are arranged centrally around the axis of the ingot and with the central zone enclosing any "blow hole" cavities that may occur in the ingot.

A still further object of the present invention is an article of manufacture having 60 a metal body with all sides thereof chilled and with any "blow hole" openings that occur located in the middle central axis and remote from the ends thereof.

A still further object of the present invention is an ingot of steel or the like comprising a body portion having zones of crystallization arranged as cups on one side of the ingot and as closed areas on the other side thereof and with "blow hole" openings 65 substantially in the middle of the ingot.

Other and further objects of the present invention will in part be obvious and will in part be pointed out hereinafter by reference to the accompanying drawings forming a part of this application and wherein like parts are designated by like characters throughout the several figures thereof.

Realizing that the present invention may be embodied in and practiced by other means than those specifically shown and described, I desire such disclosure to be understood as illustrative and not in the limiting sense.

Figure 1 illustrates the first period in the method of carrying out the process and shows crystallization building up in the bottom and sides of the mold;

Figure 2 illustrates the second period in which the pouring is finished and crystallization has begun at the top of the ingot;

Figure 3 illustrates the third period when the mold is turned to 180 degrees on its longitudinal axis.

Figure 4 illustrates the 4th period when all of the metal in the ingot has crystallized;

Figure 5 illustrates one form of mold for carrying out the present invention;

Figure 6 illustrates a transverse section through the middle of an ingot made in accordance with the present invention;

Figure 7 illustrates the operation of the 5 mold when the cover and ingot are dropped.

Heretofore in the art of casting steel ingots from "blow hole" steel, that is steel having a considerable gaseous content, difficulties have been encountered, particularly 10 where the casting was done in a covered mold. Where the ingot was cast in a horizontal covered mold the metal chilled on the long sides, the bottom and the top, as well as the ends of the ingot, since the 15 first metal run into the mold covered these portions first and therefore had a longer time to chill. Immediately gases began to be released as the metal crystallized and these gases escaped through the top surface 20 of the metal until the mold was sufficiently filled so that the metal touched the cover, or top. As soon as the top was reached a chilled skin was formed over the molten metal and the solidified metal grew 25 in all directions from the chilled portions of the mold, except under the bubbles, toward the central molten mass. Those surfaces which were first in contact with the mold, because of the longer contact time, naturally 30 built up more crystallization than the surfaces which made contact later. Therefore the bottom being the first in contact had a thicker solidified portion than either the top or the sides. The gases tending to escape 35 from the cooling steel being lighter than the steel, moved upwardly and were entrapped in the ingot beneath the upper skin thereof. Under normal conditions these bubbles formed subcutaneous cavities which would 40 break out in rolling and permit air to strike the hot side walls of the cavity and oxidize the same, so that the cavities were not likely to weld together during rolling operation. Where the metal was particularly "wild" the 45 bubbles tended to coalesce and finally reach such proportions as to cause large subcutaneous "blow holes" which caused the bloom to show scabs, "cold shuts" and other serious defects which rendered the metal unsuitable 50 for many purposes. These subcutaneous "blow holes" are a great detriment, whereas "blow holes" deeply seated in the body of the ingot are relatively harmless because such "blow holes" may be closed and welded together in rolling operations before any air strikes the side walls of such "blow holes." The gas entrapped in such deep seated "blow holes" is absorbed in the surrounding metal 55 when the ingot is highly heated and rolled 60 into a bloom.

The present invention overcomes the difficulties of the known art by the method and apparatus which will later be described in detail and wherein the gas bubbles are 65 caused to collect in the middle of the ingot

and are sufficiently deeply embedded in solid metal to prevent breaking out in rolling so that the cavities may be welded together as has been found to be possible and highly desirable. In carrying out the present invention the teeming operation is carried on slowly, preferably in a horizontal mold, so that crystallization builds up from the bottom and the side walls to a considerable thickness before the molten metal comes into contact with the chilled cover, which seals the ingot against further discharge of gases. At this point both the gas escape and the "runner" are chilled by placing cold bodies 70 against the same providing these portions have not chilled sufficiently by naturally cooling; the "fountain" having been removed before the "runner" is chilled. From this time on expelled gases are trapped 75 in the still molten steel as crystallization is growing from all of the various interior surfaces of the chilled steel except those surfaces around the "blow holes," since the presence of the gas bubbles prevent any supply of liquid metal adding to the thickness of the thin metal over the "blow holes." In order to remove these gas bubbles from 80 beneath the top, I invert the mold, that is, in a horizontal mold I turn the mold through 180 degrees around its longitudinal axis. The thick bottom now becomes the new top and the old thin top now becomes the new bottom. The bubbles which were sealed in 85 next to the original top now rise upwardly and are entrapped in the bottom of the inverted cup formed of the chilled metal that has crystallized over the bottom and sides of the mold. These bubbles are now embedded a safe distance from the ingot surfaces and the liquid metal settles into contact with the inner chilled surface of the 90 new bottom so that crystallization may grow rapidly from this new bottom upwards. The old subcutaneous "blow holes" have 95 disappeared and new deep seated "blow holes" have formed about the middle axial line of the ingot. It will be evident that the thickness of the original bottom crystallization that may be allowed to form, before the ingot is turned over, is such that may 100 be closely controlled as soon as the time of teeming and crystallization for any particular set of conditions are established. It will also be apparent that the rate of growth 105 of crystallization will be affected by the amount of "superheat" which the metal may have at the moment of teeming. These factors are readily recognized for any particular mold and metal so that the above 110 described results may be closely approximated. In carrying out this process I prefer the ingot shall be shaped after the manner set forth in my application S. N. 405,977 filed the 25th day of August, 1920. An ingot thus cast has a smooth chilled 115 120 125 130

outside surface, including the chilled ends, and such "blow holes" as are in the ingot, are harmless because of being deeply seated in the ingot. There are no parts except the 5 "runners" and the "risers" which need be broken off so that therefore the entire ingot may be rolled immediately into a bloom which requires no cropping, and so far as the ingot itself is concerned blooming will show 100% efficiency.

Reference will now be made to the drawings and more especially to Figures 5 and 7 which illustrate a horizontal two part mold as being a preferred form for carrying out 15 the present invention. It is recognized that multi-part molds may be used where desired and furthermore it is also recognized that the present method is not necessarily confined to being carried out in horizontal 20 molds. Where a two part horizontal mold is used the body portion 1 may be provided with a suitable chill cover 2, which may be provided with clamp lugs 4, that are arranged adjacent clamp lugs 5 on the body 25 portion. Suitable clamps 6 are adapted to be driven over the lugs and thus securely lock the cover in position. The cover also is provided with an opening 8 through which the "runner" 9 may extend and a "fountain" 30 10 may be mounted adjacent the "runner" to direct molten metal into the mold. Preferably the opposite end of the mold is provided with a "riser" 11 which may be partly within the cover and partly within the body 35 portion. The ends of the body portion are also preferably provided with trunnions 12 and 14 and these trunnions are mounted on suitable rails or stands 15 and 16 respectively. The trunnions may be provided with 40 flat surfaces 17 and 18 which tend to stabilize the mold when in either erect or inverted position. When the mold is filled with steel the whole device becomes substantially a solid mass of metal of which the 45 longitudinal gravity axis may be easily found and the trunnions may be located with reference to this axis so that a relatively small amount of force is required to turn the mold over on the said axis through 50 180 degrees. When the mold is filled with molten steel the axis of the filled mold substantially coincides with the axis of the trunnions and the center of gravity will be so located that the mold will tend to remain in either the upright or inverted position as 55 may be desired. In carrying out the method comprising the present invention the teeming operation is regulated to permit the steel to form cupped zones and to crystallize sufficiently to provide a considerable thickness 60 of metal adjacent the ends, sides, and bottom of the mold before the mold is filled sufficiently for the molten metal to contact with the chill top. It is to be noted that the steel at the bottom end chills first so 65 that the chill will originally be deepest at this portion. When the top 2 is reached throughout its entire length by molten metal the "fountain" 10 is removed and both the "riser" and the "runner" are chilled, then the mold is turned through 180 degrees. The 70 clamps 6 must be securely set in order to permit of this turning movement. After the mold has set a sufficient length of time for the ingot to be solidified, the clamps 6 may be knocked loose and the chill cover will 75 drop away, thereby permitting the ingot to fall from the mold. When the ingot and cover fall from the mold the center of gravity of the mold is above the axis of the trunnions because the mold now comprises 80 an empty metal trough with the bottom up- 85 permost. This tends to cause the mold to right itself automatically for a new casting operation and at the same time causes the mold to move away from over the ingot so that the latter can be easily removed.

As previously stated, the present process is particularly adapted to melted steel which carries a relatively large amount of gas and which is generally known in the art as "blow 90 hole" steel, although it may be carried out with other types and kinds of metals.

Figure 6 indicates a mid-cross-section through an ingot according to the present invention and it will be noticed that a series 95 of isocrystallization zones A are substantially cup shaped and terminate adjacent the upper side edges of the ingot while the isocrystallization zones B which form when the mold is inverted are substantially closed 100 around the "blow hole" cavities C that are located in the middle portion of the ingot.

Having described my invention, I claim:

1. The method of casting steel ingots or the like, which comprises pouring molten steel into a horizontal chill mold and permitting the steel to partly solidify to form a long narrow cup having a thick solidified wall enclosing the molten steel, continuing the pouring until said mold is filled, chilling 110 the long top surface of the molten steel in the mold to provide a solidified sheet enclosing the molten steel, and turning the mold upon its longitudinal axis to cause the gases from the cooling molten steel to collect 115 against the thick solidified wall whereby cavities formed in the ingot are deep seated therein.

2. The method of casting steel ingots in a horizontal covered chill mold which comprises pouring molten steel slowly into said mold to permit crystallization of the steel against the long bottom and shallow sides of the mold, whereby the steel will cool sufficiently to form thick walls of solidified steel 120 within which the molten steel is held, then filling the mold with molten steel and causing the same to contact with the chill cover whereby the molten steel in the mold is enclosed in a crystallized shell which entraps 125 130

gases expelled from the molten steel while crystallizing and then rotating the mold through less than 360 degrees upon its longitudinal axis to cause the gases to collect 5 against a thick side wall of the shell.

3. The method of casting steel ingots in a substantially horizontal covered chill mold which comprises slowly pouring the steel into the mold, causing the steel to contact 10 with the chill cover whereby the molten steel is enclosed in a solidified shell, and then inverting the mold upon its longitudinal axis and permitting the ingot to completely solidify while in inverted position.

15 4. The method of casting steel ingots and the like from blow hole steel which comprises running the steel into a horizontal covered chill mold and permitting the steel to solidify sufficiently to provide a solidified 20 wall having a thickness which approximates one half of the transverse dimension of the ingot through a mid-section thereof, then filling the mold with molten steel and permitting the top surface thereof to form a 25 solidified skin enclosing the non-crystallized steel, and then inverting the mold so that the thickened wall becomes the top thereof, and permitting the ingot to completely solidify while in inverted position.

30 5. The method of casting steel ingots and the like from blow hole steel which comprises running the steel into a covered chill mold having a runner at one end and a riser at the other end and permitting the steel to 35 solidify sufficiently to provide a solidified wall having a thickness which approximates one half of the transverse dimension of the ingot through a mid-section thereof, then filling the mold with molten steel and permitting 40 the top surface thereof to chill to form a solidified skin enclosing the non-crystallized steel, and then inverting the mold so that the thickened wall becomes the top thereof, and permitting the ingot to completely 45 solidify while in inverted position.

6. In the art of molding steel ingots, a mold, a removable cover on said mold, a pair of tracks, means on said mold to cause same to traverse said tracks from filling 50 position to a dumping position, the parts being arranged to cause the mold to tend to move away from dumping position when the cover is removed.

7. In the art of molding steel ingots, a 55 horizontal mold, a removable cover on said mold, removable locking means for the cover, a pair of tracks, means on said mold to cause same to traverse said tracks from filling position to a dumping position, the 60 parts being arranged to cause the mold to tend to move away from dumping position when the cover is removed.

8. In the art of molding steel ingots, a 65 mold, a removable cover on said mold, a pair of tracks, means on said mold to cause

same to be inverted and to traverse said tracks from filling position to a dumping position, the center of gravity of the inverted mold being above the axis of rotation thereof to cause the mold to tend to move away from dumping position when the cover is removed. 70

9. In the molding art, a horizontal ingot mold, a pair of tracks on which said mold is adapted to be rolled from filling position 75 to dumping position, the parts being constructed and arranged to cause said mold to tend to automatically return to filling position when the ingot is removed at the dumping position.

10. In the molding art, an ingot mold, a pair of tracks on which said mold is adapted to be rolled from filling position to dumping position, the parts being constructed and arranged to cause said mold to tend to 85 automatically move away from dumping position when the ingot is removed at the dumping position, whereby the ingot is clear of vertical obstructions so that the ingot may be easily removed. 90

11. In the molding art, a horizontal mold, trunnions on the ends of the mold, tracks on which the trunnions are adapted to roll, the center of mass of said mold being adjacent the axis of said trunnions, and a removable part attached to said mold in such manner that said center of mass is raised above said axis when said part is removed to cause the mold to tend to roll on said tracks when said part is removed. 95

12. In the art of molding steel ingots, a mold, a cover for said mold, a pair of tracks, trunnions on said mold and adapted to roll on said tracks to invert said mold for dumping the ingot and to cause a transitory 105 movement of said mold along said tracks from a filling position to a dumping position.

13. As an article of manufacture, a substantially horizontal ingot mold comprising 110 a body portion, a chill cover for said body portion, means to lock said cover in position on said body portion, and supporting trunnions for facilitating inverting said mold.

14. As an article of manufacture, a substantially horizontal ingot mold comprising 115 a body portion, a chill cover for said body portion, means to lock said cover in position on said body portion, supporting trunnions for facilitating inverting said mold, 120 and a track upon which said trunnions are adapted to roll.

15. As an article of manufacture, a substantially horizontal ingot mold comprising 125 a body portion, a chill cover for said body portion, means to lock said cover in position on said body portion, supporting trunnions for facilitating inverting said mold, and a track upon which said trunnions are adapted to roll, with the center of gravity

- being adjacent the axis of the trunnions when the mold is filled with steel and being between the axis of the trunnions and the bottom of the mold when the cover is removed and the mold is empty.
16. As an article of manufacture, a horizontal chill mold for casting steel ingots comprising a body portion, a chill cover for said body portion, means to lock said chill cover in position, and trunnions mounted on the ends of said body portion with the axis of the trunnions substantially passing through the center of gravity of said mold when the mold is filled with molten steel.
17. In the art of molding steel ingots, a mold, a cover for said mold, a support, trunnions on said mold and adapted to roll on said support to invert said mold for dumping the ingot and to cause a translatory movement of said mold along said support from a filling position to a dumping position.
18. As an article of manufacture, an ingot cast from blow hole steel and comprising cuffed isocrystallization zones on one side of said ingot and enclosed isocrystallization zones on the other side of said ingot with gas formed cavities adjacent the minimum cuffed zone.
19. As an article of manufacture, an ingot cast from blow hole steel and comprising cuffed isocrystallization zones on one side of said ingot and enclosed isocrystallization zones on the other side of said in-
- got with all surfaces of the ingot chilled and with gas formed cavities adjacent the minimum cuffed zone.
20. As an article of manufacture, an ingot of steel or the like having cuffed zones of isocrystallization on one side thereof and closed zones of isocrystallization within the cuffed zones and gas formed cavities within the minimum closed zone.
21. As an article of manufacture, an ingot of steel or the like having cuffed zones of isocrystallization on one side thereof and closed zones of isocrystallization within the cuffed zones.
22. The method of casting steel ingots or the like which consists in pouring the molten metal into a horizontally disposed chill mold, allowing the metal to partly solidify, continuing the pouring until the mold is filled, then chilling the top surface to form a shell over the molten metal, and finally inverting the mold upon its longitudinal axis and allowing the ingot to solidify in its inverted position.
23. In a horizontal ingot mold apparatus, a body portion, a chill cover for said body portion, a support, and trunnions on said body portion to roll on said support to invert said body portion, said trunnions being arranged on the body portion to move same along said support from a dumping to a filling position when the cover is removed and the mold is empty.

RAY G. COATES.